

## WATER-SOLUBLE CORROSION INHIBITORS

Walter G. Toekelt, Downers Grove, Ill., assignor, by mesne assignments, to Universal Oil Products Company, Des Plaines, Ill., a corporation of Delaware

No Drawing. Application March 26, 1958  
Serial No. 724,202

6 Claims. (Cl. 21—2.7)

This invention relates to novel water-soluble corrosion inhibitors and to the use thereof in preventing corrosion of metallic surfaces upon contact with water.

Corrosion of metallic surfaces, particularly iron and steel, in contact with fresh or salt water or various aqueous solutions, results in a serious economical loss. There is an urgent need for, and the present invention provides, improved water-soluble corrosion inhibitors which will retard and/or prevent such corrosion.

While the novel inhibitors of the present invention may be used in any system wherein water or aqueous solutions contact metallic surfaces, the following specific examples are set for as illustrative, but not limiting, instances in which the inhibitors of the present invention are useful. Storage tanks, pipe lines and the like containing petroleum oils or other organic compounds generally contain water which causes corrosion of the metallic surfaces. For example, in storage tanks the water settles to the bottom and causes corrosion of the internal surfaces of the storage tank. The water-soluble corrosion inhibitor of the present invention will dissolve in the water phase and will serve to retard and/or prevent such corrosion. Another example is in the stamping, rolling or other working of metal in which a water stream is sprayed or otherwise used as a coolant. Because these operations are effected at high temperature, the cooling water often causes extensive corrosion. Such corrosion is avoided by incorporating the corrosion inhibitor of the present invention in the water spray. Still another application is in the salt-ice water solutions used as refrigerants, for example, in railroad cars, trucks, etc. When used in railroad cars, the salt solution not only effects corrosion of the railroad cars, but also drips onto the rails and causes corrosion thereof. It is readily seen that such corrosion is a serious economical problem because it requires frequent replacement of rails, which is expensive both in manpower and in material cost. Still other applications include boiler water, acid solutions such as pickling solutions, etc.

The novel corrosion inhibitors of the present invention are reaction products of a tetrahydroxyalkyl alkylenepolyamine with phytic acid. A particularly preferred tetrahydroxyalkyl alkylenepolyamine for use in the present invention is  $N,N,N',N'$ -tetrakis-(2-hydroxyethyl)-ethylenediamine. In the interest of simplicity, this compound is referred to in the present specification and claims as tetrahydroxyethyl ethylenediamine. Other tetrahydroxyalkyl alkylenepolyamines include  $N,N,N',N'$ -tetrakis-(hydroxymethyl)-ethylenediamine,  $N,N,N',N'$ -tetrakis-(2-hydroxypropyl)-ethylenediamine,  $N,N,N',N'$ -tetrakis-(3-hydroxypropyl)-ethylenediamine,  $N,N,N',N'$ -tetrakis-(2-hydroxybutyl)-ethylenediamine,  $N,N,N',N'$ -tetrakis-(3-hydroxybutyl)-ethylenediamine,  $N,N,N',N'$ -tetrakis-(4-hydroxybutyl)-ethylenediamine,  $N,N,N',N'$ -tetrakis-(5-hydroxybutyl)-ethylenediamine, etc.,  $N,N,N',N'$ -

5 tetrakis-(hydroxymethyl)-propylenediamine,  $N,N,N',N'$ -tetrakis-(2-hydroxyethyl)-propylenediamine,  $N,N,N',N'$ -tetrakis-(2-hydroxypropyl)-propylenediamine,  $N,N,N',N'$ -tetrakis-(3-hydroxypropyl)-propylenediamine,  $N,N,N',N'$ -tetrakis-(2-hydroxybutyl)-propylenediamine,  $N,N,N',N'$ -tetrakis-(3-hydroxybutyl)-propylenediamine,  $N,N,N',N'$ -tetrakis-(4-hydroxybutyl)-propylenediamine,  $N,N,N',N'$ -tetrakis-(2-hydroxypentyl)-propylenediamine,  $N,N,N',N'$ -tetrakis-(3-hydroxypentyl)-propylenediamine,  $N,N,N',N'$ -tetrakis-(4-hydroxypentyl)-propylenediamine,  $N,N,N',N'$ -tetrakis-(5-hydroxypentyl)-propylenediamine, etc.,  $N,N,N',N'$ -tetrakis-(hydroxymethyl)-butylenediamine,  $N,N,N',N'$ -tetrakis-(2-hydroxyethyl)-butylenediamine,  $N,N,N',N'$ -tetrakis-(2-hydroxypropyl)-butylenediamine,  $N,N,N',N'$ -tetrakis-(3-hydroxypropyl)-butylenediamine,  $N,N,N',N'$ -tetrakis-(4-hydroxybutyl)-butylenediamine,  $N,N,N',N'$ -tetrakis-(5-hydroxybutyl)-butylenediamine, etc. Here again, in the interest of simplicity, these compounds are being referred to in the present specification and claims by the name of tetrahydroxyalkyl alkylenepolyamine.

While the tetrahydroxyalkyl alkylenepolyamines generally are preferred, it is understood that similarly substituted dialkylenetriamines and particularly diethylenetriamine and dipropyleneetriamine, trialkylenetetraamines and particularly triethylenetetraamine and tripropylenetetraamine, tetraalkylene pentaamines and particularly tetraethylenepentaamine and tetrapropylenepentaamine, etc. may be employed for reaction with phytic acid but not necessarily with equivalent results.

40 The reaction of the tetrahydroxyalkyl alkylenepolyamine and phytic acid is effected using about 0.5 to about 6 mol proportions of the tetrahydroxyalkyl alkylenepolyamine per 1 mol proportion of phytic acid. The reaction readily is effected at atmospheric temperature although in some cases elevated temperature, which generally will not exceed about 100° C., may be employed. When higher temperatures are used, the reaction preferably is effected under superatmospheric pressure in order to maintain the reactants in substantially liquid phase.

45 While the tetrahydroxyalkyl alkylenepolyamine and phytic acid may be reacted under anhydrous conditions, for ease of handling and reacting, generally aqueous solutions thereof are utilized. The aqueous solution may contain from 10% to about 80% by weight of the active component. As another advantage to utilizing aqueous solutions of the reactants, the reaction product is recovered as an aqueous solution and the aqueous solution is utilized as a corrosion inhibitor, without the additional time and expense otherwise necessary to separate the reaction product from the aqueous solvent. When a more dilute solution is desired, additional water may be commingled with the reaction product in order to form a final solution of the desired concentration.

50 60 As hereinbefore set forth, the reaction product is recovered and used as an aqueous solution. However, when desired, the reaction product may be separated from the aqueous solvent in any suitable manner, and the reaction product utilized as such or as a solution in other solvents 65 as, for example, alcohols, ketones, aldehydes, etc.

65 The exact composition of the reaction product has not been determined. Without any intention of being limited thereto, it is believed that the reaction product comprises a salt, although it may consist of or comprise esters, or mixtures of salts and esters. Regardless of the specific composition of the reaction product, it has been

determined that the reaction product is an effective corrosion inhibitor, and the same is being disclosed and claimed herein for such use.

As hereinbefore set forth, the reaction product prepared in the above manner is utilized as a water soluble corrosion inhibitor. The reaction product is incorporated in water, aqueous solutions or substrates containing water in a sufficient concentration to effectively retard corrosion of metallic surfaces. Generally, it will be utilized in a concentration of below about 1% by weight of the water, aqueous solution or substrate containing water, and more particularly in a concentration within the range of from about 0.001% to about 1% and still more particularly of from about 0.01% to about 0.5% by weight thereof, although higher concentrations may be employed when excessive corrosion is encountered. It is understood that the corrosion inhibitor may be used in conjunction with other additives which are incorporated in the substrate for various reasons.

The following examples are introduced to illustrate further the novelty and utility of the present invention but not with the intention of unduly limiting the same.

The reaction product of the present invention was evaluated as a corrosion inhibitor by the following method. A 600 cc. beaker was used as the reaction vessel and 300 cc. of a 5% sodium chloride solution containing the inhibitor was introduced into the beaker. A 0.5" x 3" x 1/8" mild steel strip was inserted in the beaker and held in a horizontal position with one end resting on a glass rod. The sodium chloride solution was stirred by a single blade stirrer revolving at 250 r.p.m. Air was continuously bubbled in at the rate of 5.6 liters per hour.

When evaluated in the above manner, a steel strip, after six hours exposure in a brine not containing inhibitor, showed a weight loss of 20 mg.

#### Example I

The reaction product of this example was prepared by reacting tetrahydroxyethyl ethylenediamine with phytic acid. To a solution of 1.4 gms. of phytic acid in 10 gms. of water, 2 gms. of tetrahydroxyethyl ethylenediamine (N,N,N',N'-tetrakis-(2-hydroxyethyl) - ethylenediamine) was added at room temperature. The reaction was slightly exothermic. The reaction product was a clear solution having a slight yellowish hue.

The reaction product, in a 50% by weight aqueous solution, was evaluated in another sample of the brine described above and in the same manner as described therein. The reaction product was used in a concentration of 0.02% by weight of active ingredient (0.04% by weight of aqueous solution). When evaluated in this manner the steel strip lost only 2.2 mg. It will be noted that the reaction product was very effective in retarding corrosion of the metal.

#### Example II

In this example the reaction product was prepared in the absence of water. Upon mixing at room temperature of the tetrahydroxyethyl ethylenediamine and phytic acid, heat is given off and a thick, gelatinous material is formed. Upon boiling, this material was converted into a tan glass. This product is soluble in water and, when prepared as an aqueous solution, is evaluated in the same manner

as described in Example I for use as a corrosion inhibitor.

#### Example III

The corrosion inhibitor of this example is prepared by reacting at room temperature 1 mol proportion of N,N,N',N' - tetrakis - (2 - hydroxyethyl) - 1,3 - diamino propane with 1 mol proportion of phytic acid. The reactants are used as aqueous solutions of 50% concentration, and the reaction product is recovered as an aqueous solution. The reaction product is evaluated as a corrosion inhibitor in the same manner as described in Example I. The loss in weight of the steel strip is reduced considerably below the 20 mg. loss obtained in the absence of the inhibitor.

I claim as my invention:

1. The method of retarding corrosion of a ferrous metal upon contact with water which comprises effecting said contact in the presence of a water-soluble corrosion inhibitor comprising the product formed by the reaction of from about 0.5 to about 6 mol proportions of a tetrahydroxyalkyl alkylenepolyamine with 1 mol proportion of phytic acid, the first-mentioned compound containing from 2 to 5 amine groups per molecule and having from 1 to 5 carbon atoms in each of the alkyl groups and from 2 to 4 carbon atoms in the alkylene group.

2. The method of retarding corrosion of a ferrous metal upon contact with water which comprises effecting said contact in the presence of a water-soluble corrosion inhibitor comprising the product formed by the reaction of from about 0.5 to about 6 mol proportions of tetrahydroxyethyl ethylenediamine with 1 mol proportion of phytic acid.

3. The method of retarding corrosion of a ferrous metal upon contact with water which comprises effecting said contact in the presence of water-soluble corrosion inhibitor comprising the product formed by the reaction of from about 0.5 to about 6 mol proportions of tetrahydroxyethyl propylene diamine with 1 mol proportion of phytic acid.

4. Water containing as a corrosion inhibitor the product formed by the reaction of from about 0.5 to about 6 mol proportions of a tetrahydroxyalkyl alkylenepolyamine with 1 mol proportion of phytic acid, the first-mentioned compound containing from 2 to 5 amine groups per molecule and having from 1 to 5 carbon atoms in each of the alkyl groups and from 2 to 4 carbon atoms in the alkylene group.

5. Water containing as a corrosion inhibitor the product formed by the reaction of from about 0.5 to about 6 mol proportions of tetrahydroxyethyl ethylenediamine with 1 mol proportion of phytic acid.

6. Water containing as a corrosion inhibitor the product formed by the reaction of from about 0.5 to about 6 mol proportions of tetrahydroxyethyl propylene diamine with 1 mol proportion of phytic acid.

#### References Cited in the file of this patent

#### UNITED STATES PATENTS

- |           |                  |               |
|-----------|------------------|---------------|
| 2,626,238 | Arts             | June 20, 1953 |
| 2,697,118 | Lundsted et al.  | Dec. 14, 1954 |
| 2,755,304 | Bersworth et al. | July 17, 1956 |